

## UNITED STATES PATENT OFFICE

1,932,050

## EXPLOSIVE COATING MATERIAL

Charles P. Spaeth, Woodbury, N. J., assignor to  
E. I. du Pont de Nemours & Company, Wil-  
mington, Del., a corporation of Delaware

No Drawing. Application November 20, 1931  
Serial No. 576,435

11 Claims. (Cl. 52—11)

My invention relates to a new and improved coating material for explosive compounds and explosive ingredients and more particularly to an explosive coating material comprising tri-

5 methylol ethyl methane trinitrate.

In the high explosive industry, it is a frequent practice to use coated ingredients in order to modify and control the physical characteristics of such ingredients. For example, coated ammonium nitrate has been in use for a great many years. In this case, the ammonium nitrate granules are covered with a thin coating of paraffin, petrolatum, or other suitable material. The object of such coating on the ammonium nitrate is 10 to reduce the tendency of the ammonium nitrate to take up moisture from the surrounding atmosphere, due to the great hygroscopicity of the material. The use of the coating material has brought about many advantages. Similarly other 15 coating materials have been used both for protection against moisture and for other reasons. Ammonium nitrate has frequently been coated with trinitrotoluene for example, in such manner that the coating not only gave protection 20 against moisture but also increased the sensitivity of the ammonium nitrate.

One of the objects of my invention is to bring about a coating of ingredients for explosive compositions by a new and improved material, which 25 is itself an explosive. Another object is the use of a compound as a coating material for ingredients of explosive compositions, which will reduce their tendency to absorb moisture.

A further object is the use of a compound as 30 a coating material, having itself such properties as an explosive that relatively insensitive explosive materials will have increased sensitiveness. A still further object is the use of a compound which, when distributed as a coating on explosives of unduly high sensitiveness, will bring 35 about a desensitizing effect. Another object is the use of a compound as a binder in the preparation of free running granules from a finely divided, non-free running explosive material; or 40 as a binder for holding in intimate contact a mixture of several ingredients used in explosive compositions. Further objects will be apparent as my invention is more fully described herein- 45 after.

50 In my copending application, Serial No. 576,434, filed November 20, 1931 I have disclosed the new chemical compound trimethylol ethyl methane trinitrate which has highly valuable properties as an explosive compound. This substance is ob- 55 tained by the nitration, in any suitable way, of

the trihydroxy compound, trimethylol ethyl methane. The nitrated product has the following formula:—



60

I have discovered that trimethylol ethyl methane trinitrate is highly desirable as a coating material for other ingredients of explosives and particularly so for other explosive compounds. Because of its intermediate degree of sensitiveness, it is adapted for use either as a coating for insensitive materials, in which case it functions as a sensitizing agent, or as a coating for materials that are so highly sensitive as to be undesirable for use alone, in which case it serves as a desensitizing agent.

As for an example of the use of trimethylol ethyl methane trinitrate as a coating material 75 for insensitive materials, I will cite its use in the coating of ammonium nitrate. Trimethylol ethyl methane trinitrate has the necessary properties for use as a coating ingredient, having as 80 it does a waxy nature and a melting point of about 48° C. As a result of this, it is readily applied as a surface coating to the granules of ammonium nitrate. While it has all the advantages of paraffin and similar coating materials as a waterproofing agent, trimethylol ethylmethane trinitrate is free from the disadvantages of paraffin. While paraffin has a decided desensitizing effect 85 when applied as a coating material, trimethylol ethyl methane trinitrate is itself an explosive compound of an intermediate degree of sensitiveness so that it both protects ammonium nitrate against moisture and increases its sensitiveness. Likewise paraffin, and other of the organic coating materials commonly used for coating explosive ingredients, are very deficient in oxygen. 90 Trimethylol ethyl methane trinitrate, however, is only slightly deficient in oxygen, hence considerable more of this material may be used as a coating when desirable without disturbing the balance of oxygen for complete combustion of the explosive mixture. Trimethylol ethyl methane trinitrate may be used to coat other insensitive ingredients of dynamite, as for example sodium nitrate, potassium nitrate, calcium nitrate, urea nitrate, ammonium perchlorate, and 95 the like.

Trimethylol ethyl methane trinitrate may also be used to advantage in the coating of explosive materials having too high a degree of sensitiveness for safe use in practice. Trimethylol ethyl 100

105

110

methane trinitrate has itself an intermediate degree of sensitiveness so that its use as a coating material confers its own degree of sensitiveness on the ingredient coated. An illustration of such use lies in its application as a coating material for compounds adapted for use as primary detonating compounds, as well as materials suitable for use as ignition ingredients in blasting caps, which, however, are undesirably sensitive for use by themselves, as for example hexamethylene-triperoxidatediamine, trinitrotriazidobenzene, and like compounds.

A further illustration of the use of trimethylol ethyl methane trinitrate as a coating ingredient of the second class, is its use with pentaerythrite tetranitrate. This compound is used frequently with considerable satisfaction as the filling material for detonating fuse. However, the sensitiveness of fuses filled with pentaerythrite tetranitrate is undesirably high for use in rough work where the material may be exposed to shock and heavy blows. The coating of the pentaerythrite tetranitrate core of such fuse with trimethylol ethyl methane trinitrate obviates the above difficulties, and gives a satisfactory fuse material.

It is well known that certain explosive ingredients are prepared in such a way that they comprise finely divided, non-free running, dusty materials which are inferior as constituents of explosive compositions on account of the difficulty in mixing, loading and packing, and which are dangerous because of the dust hazard. I find that my new explosive coating material may be used quite successfully in removing these difficulties. Dusty, non-free running materials, when mixed in suitable amounts with trimethylol ethyl methane trinitrate, may be made into granules or pellets of a desirable size, which are free running, non-dusty and suitable for mixing, loading, and packing as a constituent of any explosive composition. As examples of this, I may mention nitrostarch, pentaerythrite tetranitrate, cyclotrimethylene trinitramine, tetryl, and like compounds.

Likewise, it is often desirable to combine in a more intimately associated form a mixture of several explosive ingredients. This has the desirable feature of preventing the segregation of a mixture of materials having varying densities. It has the additional advantage of promoting more rapid and more complete combustion of this mixture, with consequent improvement in explosive propagation. It likewise allows an improved method of governing the size and form of the grains or pellets, with the result that the properties of the explosive may be modified and improved. For example, I may bind together a mixture of ammonium nitrate, sodium nitrate, and an organic combustible material for use, by itself or with other ingredients, as a blasting explosive. Again it is useful in preparing a mixture suitable as an ignition agent in caps which

may comprise, for example, lead sulphocyanate, potassium chlorate, and ground smokeless powder.

It will be understood that in the use of trimethylol ethyl methane trinitrate as a coating material for explosive ingredients and compounds, the thickness of the coating will vary in accordance with the necessities of the case. A coating should be used of sufficient thickness so that the desired degree of sensitiveness is obtained for the material coated.

It will be further understood that the coating may be applied in the form of liquid trimethylol ethyl methane trinitrate at an increased temperature for example 50-60° C., or the coating material may be dissolved in a suitable solvent or mixture of solvents and applied at room temperature, the solvent or solvents being subsequently removed by evaporation.

While I have described my invention in detail in the foregoing, I wish it to be understood that many variations may be made without departure from the spirit of the invention, and that I do not intend to be limited except as indicated in the following patent claims:

I claim:

1. A new composition of matter comprising an ingredient of an explosive composition coated with trimethylol ethyl methane trinitrate.

2. A new composition of matter comprising an inorganic ingredient of an explosive composition coated with trimethylol ethyl methane trinitrate.

3. A new composition of matter comprising an inorganic explosive salt coated with trimethylol ethyl methane trinitrate.

4. A new composition of matter comprising ammonium nitrate coated with trimethylol ethyl methane trinitrate.

5. A new composition of matter comprising an organic ingredient of an explosive composition coated with trimethylol ethyl methane trinitrate.

6. A new composition of matter comprising an explosive compound coated with trimethylol ethyl methane trinitrate.

7. A new composition of matter comprising an organic explosive compound coated with trimethylol ethyl methane trinitrate.

8. A new composition of matter comprising hexamethylenetriperoxidatediamine coated with trimethylol ethyl methane trinitrate.

9. A new composition of matter comprising an explosive mixture, the ingredients of which are coated with trimethylol ethyl methane trinitrate.

10. An explosive composition comprising a mixture of a sulfocyanate, an oxidizing agent, and a fuel, said ingredients being coated with trimethylol ethyl methane trinitrate.

11. An explosive composition comprising lead sulfocyanate, potassium chlorate, and ground smokeless powder, said ingredients being coated with trimethylol ethyl methane trinitrate.

CHARLES P. SPAETH.